

## UNITED STATES PATENT OFFICE

2,138,773

## PROCESSES FOR REFINING HYDROCARBON OILS BY MEANS OF BENZOL DERIVATIVES

Ernst Terres, Berlin, Germany, and Josef Moos, New York, and Erich Saegebarth, Jackson Heights, N. Y., assignors to Edeleanu Gesellschaft, m. b. H., a corporation of Germany

No Drawing. Application October 25, 1937,  
Serial No. 170,969

## 5 Claims. (Cl. 196—13)

This invention relates to the refining of hydrocarbon oils, such as mineral oils, coal tar or bituminous coal tar oils, by means of selective solvents which have the characteristics of dissolving certain undesirable fractions present in hydrocarbon oils for producing oils suitable for lubricating purposes, and is a continuation in part of our application Serial No. 12,527, filed March 22, 1935, for Process for refining hydrocarbon oils by means of ketones, organic acids, organic anhydrides, organic oxides, alcohols, and ethers.

Although not much is known about the actual constitution of the individual components present in hydrocarbon oils, it is understood that cuts or fractions which are heavy enough for lubricating stock contain representatives of the aromatic, hydroaromatic and unsaturated groups which are undesirable for lubricating purposes. The removal of these undesirable components by means of suitable selective solvents leaves an undissolved fraction which contains mainly paraffin-like components. These undissolved fractions or raffinates are identified by greatly improved physical and chemical specifications, such as gravity, viscosity temperature relationship, Conradson carbon and resistance against oxidation.

We have found that benzal acetone has very good selective solvent action upon hydrocarbon oils. This solvent dissolves the undesirable fractions of hydrocarbon oils as described above and produces a greatly improved raffinate. In carrying out our invention, we contact the selective solvent with the hydrocarbon oil to be treated in batch or in countercurrent using a mixing and settling equipment or a tower mixer.

The effect of our solvents upon mineral oils may be seen from the following examples.

## Example 1

A dewaxed distillate produced from a Mid-Continent crude with properties as shown in the following table, was extracted at 115° F. in two successive treatments with 100% volume (in each treatment) of benzal acetone



having a boiling point of 504° F., and a melting point of 108° F., and after recovering the solvent

from the raffinate and extract solutions the products were found to have the following properties:

|                                  | Mid-Continent dewaxed distillate | Raffinate | Extract | 5  |
|----------------------------------|----------------------------------|-----------|---------|----|
| Yield by volume.....             | 100                              | 63.7      | 36.3    |    |
| °A. P. I.....                    | 23.0                             | 28.5      | 14.2    |    |
| Saybolt viscosity at 100° F..... | 1379                             | 709       | .....   | 10 |
| Saybolt viscosity at 210° F..... | 93.4                             | 74.7      | .....   |    |
| Viscosity index.....             | 73.7                             | 97.5      | .....   |    |
| Carbon residue.....              | 1.9                              | 0.30      | .....   |    |

Instead of employing benzal acetone as a selective solvent alone, we may use this solvent in the presence of an auxiliary solvent of the class which is miscible in any proportion with benzal acetone and not entirely miscible with the hydrocarbon oils to be extracted. This class of auxiliary solvents serves to decrease the solvent power of benzal acetone, which is the selective solvent; and to this class of auxiliary solvents belong, for example, the alcohols.

## Example 2

The following example illustrates the effect of the admixture of ethyl alcohol as an auxiliary solvent with benzal acetone for extracting a mineral lubricating oil distillate.

The same dewaxed Mid-Continent distillate as used in Example 1 was extracted with 100% plus 2×50% of a mixture containing 60 volume per cent benzal acetone and 40 volume per cent ethyl alcohol at 75° F. After each extraction the extract was separated from the raffinate layer and, after recovering the solvents therefrom the products were found to have the following properties:

|                                  | Raffinate | Extract | 40 |
|----------------------------------|-----------|---------|----|
| Yield percent by volume.....     | 78.3      | 21.7    |    |
| °A. P. I.....                    | 27.4      | 9.8     |    |
| Saybolt viscosity at 100° F..... | 79.6      | .....   |    |
| Saybolt viscosity at 210° F..... | 77.0      | .....   |    |
| Viscosity index.....             | 92        | .....   |    |
| Carbon residue.....              | 0.43      | .....   | 45 |

It will be seen from the above example that the addition of ethyl alcohol to benzal acetone decreases the solvent power of the latter substantially.

Instead of recovering the benzal acetone from the raffinate and extract solutions by distillation, we may employ a different solvent which dissolves only the benzal acetone but not the hydrocarbon fractions. From the solvent mixture containing the additional solvent, and our selective and auxiliary solvents, we may remove the additional solvent either by distillation or by the addition of water or other agents which cause it 10 to become insoluble in our selective and auxiliary solvents.

Other scopes of our invention and the action of the auxiliary solvents is explained in our co-pending applications Serial Nos. 12,526, 12,528 15 and 12,529, filed March 22, 1935.

We claim the following as our invention:

1. A process for refining hydrocarbon oils by extracting the latter with benzal acetone at suitable temperatures, to produce separation into two 20 layers, separating the layers containing respectively paraffinic and non-paraffinic constituents from each other and recovering the solvent from the layers.

2. A process for refining hydrocarbon oils by 25 solvent extraction in which benzal acetone is used in presence of an alcohol which is miscible with the selective solvent but which is not miscible, or miscible only to a small degree, with the hydrocarbon oils to be extracted, the addition of said 30

alcohol decreasing the solvent power of the selective solvents.

3. A process of refining mineral oil comprising mixing the oil with benzal acetone as selective solvent and adjusting the temperature to produce a separation into two oil containing phases, separating the phases from each other and recovering the solvent therefrom.

4. A process of refining a mineral oil comprising extracting the oil with benzal acetone as a 1 selective solvent in admixture with an auxiliary solvent to produce a separation into two phases containing relatively paraffinic and non-paraffinic constituents, separating the two phases from each other and recovering the solvents therefrom.

5. A process of refining lubricating oil, containing paraffinic and non-paraffinic constituents, comprising extracting said lubricating oil with benzal acetone as a selective solvent at a temperature of above 108 degrees Fahrenheit, to produce 2 a dissolved layer, consisting of the non-paraffinic oil constituents dissolved in the bulk of the selective solvent, and an undissolved layer, consisting of the paraffinic oil constituents saturated with the selective solvent, separating the dissolved 2 layer from the undissolved layer and removing the solvent from both layers.

ERNST TERRES.

JOSEF MOOS.

ERICH SAEGBARTH. 3